

Feb. 9, 1926.

1,571,973

H. J. SHIVELL ET AL

LEATHER BELT AND PROCESS OF PRODUCING SAME

Filed Dec. 3, 1920

FIG 1



FIG 2



Inventor  
Homer J. Shivell & Karl W. Koeniger  
By Their Attorneys  
Newell & Speer

## UNITED STATES PATENT OFFICE.

HOMER J. SHIVELL AND KARL W. KOENIGER, OF KINGSPORT, TENNESSEE, AS  
SIGNORS TO GRANT LEATHER CORPORATION, A CORPORATION OF VIRGINIA.

## LEATHER BELT AND PROCESS OF PRODUCING SAME.

Application filed December 3, 1920. Serial No. 428,160.

To all whom it may concern:

Be it known that we, HOMER J. SHIVELL and KARL W. KOENIGER, citizens of the United States, both residing at Kingsport, Tennessee, have invented certain new and useful Improvements in Leather Belts and Processes of Producing Same, of which the following is a clear, full, and exact description.

Our invention relates to an improvement in leather belts and process of producing same. Our object is to improve the construction and produce a belt which will be stronger and more efficient particularly when first applied. It is well known that the ordinary leather belt when first applied does not give its maximum tractive effect or attain its maximum efficiency. After it has been run for a while, its surface will show a somewhat mottled appearance, portions thereof being lighter than others. This is caused by the surface not contacting at all points with the pulley over which it runs, with consequent loss of efficiency. As the belt continues in use, the mottled appearance gradually disappears, due to the fact that the friction surface thereof gradually becomes "set" so as to contact to a greater extent over its entire area. The maximum tractive effect is therefore not attained in the ordinary leather belt until after a considerable period of use. We are able to produce a belt which, when new, will be more efficient and will much more nearly approach its maximum frictional efficiency, besides attaining other advantages.

An unhaired hide is not homogeneous from the upper surface down but consists of several layers having different characteristics. A section thereof is illustrated in Fig. 1, in which 1 represents the epidermis or outer layer, 2 the so-called "real skin," 3 the so-called "middle portion" and 4 the remainder or so-called "fibre." It will be understood that in the illustration the thickness of the first three layers not only with relation to themselves but with relation to the thickness of the fiber layer has been exaggerated for clarity of illustration. The epidermis and "real skin" contain pores. These are very fine passages in the "real skin" illustrated, for example at 5, which open out in the epidermis, as illustrated at 6. In them or some of them, the hair roots

indicated, for example at 7, are located. The relative size of these pores is of course greatly exaggerated in the illustration. These pores, while they are minute, are multitudinous over the entire surface, and in the aggregate leave a considerable area of the upper or contacting surface in which the leather does not actually contact with the pulley, thus losing tractive effect. Filling up such surface openings with a permanent filler increases the contacting surface of the belt as a whole, but careful tests show that when the pores are left as the hide comes to the manufacturer in unhaired condition, the presence of the pores in their original form decreases quite materially the tensile strength of the leather. We believe this is caused, at least in part, by the pores, particularly the roughly inverted-conical shape of the upper portion thereof, presenting what is in effect a multitude of embryonic cracks extending part way through the leather from the upper or contacting surface where the greatest strain occurs down into or through the upper layers. The hair side of the belt is used as the surface which contacts with the pulley, as it has been found that this is the most efficient side. The problem of producing a more efficient belt therefore presents these two apparently irreconcilable desiderata. By our method of manufacture, we have been able substantially to reconcile to a great extent these two things and produce a belt which is considerably more efficient even when new than the leather belts heretofore made.

In carrying out our invention in the manner we prefer, we remove the upper portion of the leather. This may be done by various methods but a convenient method is by splitting it as indicated diagrammatically in Fig. 2, in which 8 indicates the leather passed through between yielding rolls 9 and 10 and split by a straight-edged knife 11. This will give a smooth upper surface to the remaining portion 12. We split the leather above the lower margin of the "real skin" 2, preferably between the lower and upper margin thereof, as indicated for example at the dotted line 13 in Fig. 1. This consequently removes much, and preferably all, of the epidermis which contains the enlargements of the pores but does not remove all

the "real skin" which contains the more minute portions of the pores. It therefore retains the advantage of leaving part of the "real skin" in place for its tractive effect 6 while reducing the area of the pore openings at the surface, thus not only reducing the tendency of the surface to split under tension but increasing the area of leather which actually contacts with the pulley.

- 10 While a belt made from leather merely so split would accomplish some of the results we have attained, the belt should be internally lubricated and preferably the remaining pores of the upper surface should be 15 filled up by a filler which is of such a character as permanently to fill the pores and consequently increase the total area of the belt which contacts with the pulley. The belt may be impregnated with various oily 20 substances such as the oils or greases ordinarily used in rendering leather pliable, such for example as paraffin oil, tallow, etc. The filler for the pores may be and preferably is rubber. It may be applied in different ways to the upper surface. We, however, have found that a successful manner of applying it is to finely divide it, for example by dissolving the crude rubber in gasoline or other volatile solvent which will evaporate after having thoroughly filled the pores. The rubber obviously has a considerably higher melting point than the lubricant mentioned.

25 We prefer to mix the rubber, dissolved as above described, with the lubricant and apply the mixture to the belt, preferably by forcing it into the leather from the upper surface. This carries the lubricant and finely divided rubber through the pores. 30 The lubricant passes on into and impregnates the lower layers thoroughly and will work into all portions thereof. The filler, however, need not pass into the lower layers, as its purpose is mainly to fill up the 35 exposed pores, and as they are very minute in the "real skin," the filler will be retained mainly in the pores, filling them completely and resulting in a substantially continuous surface over the entire upper area of the belt. The rubber solvent is then allowed to 40 evaporate, leaving the pores completely filled with the rubber. The surplus may then be scraped or brushed off, leaving the upper or contacting surface smooth and without unfilled pores, yet with the general pore appearance of the hair side of the hide. The belt has considerably greater tractive effect 45 even when first applied, its tensile strength is increased, and in short it is a considerably

more efficient belt than one manufactured in 60 the ordinary manner.

We are aware that variations in the foregoing steps may be made without departing from the scope of our invention as claimed, and we therefore do not desire to be limited 65 to the exact features above described.

What we claim is—

1. The process of manufacturing leather for power transmission belts and the like, which comprises removing the epidermis, the 70 grain and a portion of the "real skin" of the leather, thereby removing that part of the leather containing the enlargements of the pores and leaving the upper surface smooth, and impregnating the remaining 75 portion of the leather with an oily lubricant, and filling up the pores in the "real skin" with a finely divided filler which has a considerably higher melting point than said lubricant, and which is of such a character as permanently to fill said pores.

2. The process of manufacturing leather for power transmission belts and the like, which comprises removing the epidermis, the 80 grain and a portion of the "real skin" of the leather, thereby removing that part of the leather which contains the enlargements of the pores and leaving the upper surface smooth, impregnating the remaining portion 85 of the leather with an oily lubricant and filling up the pores in the "real skin" with a finely divided rubber filler.

3. The process of manufacturing leather for power transmission belts and the like, which comprises removing the epidermis, the 90 grain and a portion of the "real skin," thereby removing that portion of the leather containing the enlargements of the pores and leaving the upper surface smooth, impregnating the remaining portion of the leather 95 with a mixture of an oily lubricant with a solution of rubber without other ingredients to impregnate the leather with the lubricant and to fill the pores in the "real skin" with rubber.

4. A leather belt in which the epidermis, the grain and a portion of the "real skin" have been removed, and having a smooth upper surface, the belt being impregnated with an oily lubricant and the pores in the 100 same being filled with a permanent filler which has a considerably higher melting point than said lubricant.

Signed at Kingsport, Tenn., this 26 day of November, 1920.

HOMER J. SHIVELL,  
KARL W. KOENIGER.